

## UNITED STATES PATENT OFFICE

2,268,428

## HARD METAL ALLOY

Robert W. Schlumpf, Houston, Tex., assignor to  
 Hughes Tool Company, Houston, Tex., a corporation of Delaware

No Drawing. Application November 10, 1941,  
 Serial No. 418,596

2 Claims. (Cl. 75—126)

This invention pertains to the composition of hard metal objects which are resistant to wear and abrasion.

It is an object of the invention to provide an alloy composition which may be employed in the manufacture of tools or devices which are subject to heavy wear through abrasion thereon. It may be employed in the construction of nozzles for the discharge of fluid having abrasive particles such as sand therein.

I have found that an alloy made up of elements combined together in approximately the following proportions produces a satisfactory compound of this character:

|           | Per cent               |
|-----------|------------------------|
| Carbon    | 1.50—3.50              |
| Manganese | 0.50—2.50              |
| Silicon   | 0.50—2.00              |
| Chromium  | 14.0—20.0              |
| Tungsten  | 14.0—20.0              |
| Boron     | 0.50—1.50              |
| Iron      | Balance to make up 100 |

These materials when fused together within the ranges indicated will produce a metal which is extremely hard and wear resistant and adapted to be used in the casting of tools and devices subject to extreme wear. The resulting alloy is not malleable and is best employed in the construction of devices which are not subject to heavy shock or impact.

While the proportions of the separate ingredients to be employed may be varied and still obtain fairly satisfactory results a typical composition which I have found particularly satisfactory is as follows:

|           | Per cent               |
|-----------|------------------------|
| Carbon    | 2.24                   |
| Manganese | 1.40                   |
| Silicon   | 1.19                   |
| Chromium  | 16.0                   |
| Tungsten  | 17.5                   |
| Boron     | 1.20                   |
| Iron      | Balance to make up 100 |

Devices constructed from this alloy are extremely hard and although they are particularly adapted for sand blast or bit nozzles it will be obvious that the alloy is adapted for general use in the manufacture of tools to be employed in situations where exceptional wear is encountered.

What is claimed as new is:

1. A hard ferrous metal alloy resistant to abrasion, comprising elements fused together in the following proportions:

|             | Per cent               |
|-------------|------------------------|
| Carbon      | 1.50—3.50              |
| Manganese   | 0.50—2.50              |
| Silicon     | 0.50—2.00              |
| 15 Chromium | 14.0—20.0              |
| Tungsten    | 14.0—20.0              |
| Boron       | 0.50—1.50              |
| Iron        | Balance to make up 100 |

2. A hard metal casting composed of an alloy having ingredients in approximately the following proportions:

|             | Per cent               |
|-------------|------------------------|
| Carbon      | 2.24                   |
| Manganese   | 1.40                   |
| Silicon     | 1.19                   |
| 25 Chromium | 16.0                   |
| Tungsten    | 17.0                   |
| Boron       | 1.20                   |
| Iron        | Balance to make up 100 |

ROBERT W. SCHLUMPF.

35

40